

1

3,189,629

**PROCESS FOR TREATING SYNTHETIC ESTER LUBRICANTS WITH AROMATIC ISOCYANATES OR AROMATIC THIOISOCYANATES**

Dietrich F. Hottenlocher, Philadelphia, Pa., and William M. Sweeney, Wappingers Falls, N.Y., assignors to Texaco Inc., New York, N.Y., a corporation of Delaware  
No Drawing. Filed Nov. 21, 1960, Ser. No. 70,370  
6 Claims. (Cl. 260—404.8)

This invention relates to a method of treating synthetic ester lubricating oils. More particularly it relates to a novel method of reducing the acidity and hydroxyl content of synthetic ester oils employing aromatic hydrocarbyl isocyanate or an aromatic hydrocarbyl isothiocyanate as the treating agent.

Synthetic esters are widely used as lubricating oils in engines which are subject to high temperatures such as combustion turbine engines, particularly those of the "turbo-jet" and "prop-jet" type. The reason for this is these synthetic ester oils are generally characterized by a higher viscosity index and lower pour point than mineral oils of corresponding viscosity. In addition they leave a lower percentage of carbonaceous residue than their mineral oil counterparts. Carbonaceous residue from engine oils is undesirable in that it accumulates and interferes with the operation of the engine. In addition the synthetic ester lubricants generally have higher flash points than mineral oils of equivalent viscosity thereby lessening the danger of combustion of the oil at high engine temperature operation.

The synthetic esters can be broadly described as esters of hydrocarbyl carboxylic acids and hydrocarbyl alcohols. They are high molecular weight materials of lubricating oil characteristics derived from alcohols which are usually aliphatic alcohols containing from 1 to 4 or more hydroxyl radicals and carboxylic acids which are usually aliphatic carboxylic acids containing from 1 to 4 or more carboxyl acid radicals.

Widely used synthetic ester lubricants are aliphatic esters of saturated aliphatic monocarboxylic and dicarboxylic acids containing 6-12 carbon atoms. From the standpoint of cost and availability the preferred carboxylic acids are caproic, heptoic, caprylic, pelargonic, nonylic, adipic, sebacic and azelaic acids. The mono-hydric and polyhydric aliphatic alcohols used to form the esters usually contain at least 4 carbon atoms and up to 20 or more carbon atoms. C<sub>6</sub> to C<sub>18</sub> saturated aliphatic alcohols are commonly used such as 2-ethylhexanol and 2,2-diethyl-1,3-propanediol. Ether alcohols such as 2-ethoxyethanol and monoethyl ether of diethylene glycol may also be employed in the formulation of ester oils. Alcohols containing two or more hydroxyl radicals and an absence of hydrogen on the beta carbon atom such as trimethylolethane, pentaerythritol and trimethylolpropane have proven particularly effective in formulating stable high temperature ester lubricants.

Examples of simple esters of a aliphatic carboxylic acid and alcohol are the following: diisooctyl azelate, di-2-ethylhexyl sebacate, di-2-ethylhexyl azelate, di-2-ethylhexyl adipate, dilauryl azelate, di-sec-amyl sebacate, di-2-ethylhexyl alkenyl succinate, di-2-ethoxyethyl sebacate, di-2-(2'-methoxyethoxy)ethyl sebacate, di-2-(2'-butoxyethoxy)ethyl sebacate, di-2-butoxyethyl azelate, di-2-(2'-butoxyethoxy)ethyl alkenylsuccinate, tetracaproate of pentaerythritol, triisooctanoate of trimethylolpropane and nonyl caproate.

In addition to such esters, complex ester lubricants formed by a reaction of an aliphatic polycarboxylic acid, an aliphatic polyhydroxy compound and a monofunctional aliphatic alcohol or acid are also employed as syn-

2

thetic lubricants. Complex esters of this type are described in U.S. 2,628,974. Complex esters formed by the reaction of a mixture containing stoichiometric amounts of 2-ethyl-1,3-hexanediol, sebacic acid, and 2-ethylhexanol and by reaction of a mixture containing adipic acid, diethylene glycol, and 2-ethylhexanoic acid illustrate this class of synthetic complex ester lubricating oils. Further illustrations of the complex esters are the ester reaction products of sebacic acid, trimethylolpropane and pelargonic acid; sebacic acid, trimethylolpropane, and 2-ethylhexanol; sebacic acid, trimethylolethane and hexanoic acid; and suberic acid, 1,3,5,7-octanetetraol and pentanoic acid.

The sulfur analogues of the foregoing esters are also useful as synthetic lubricants. For example, simple thioesters are illustrated by di-2-ethylhexyl thiosebacate, di-n-octyl thioadipate and the dilaurate of 1,5-pentanedithiol; sulfur analogues of complex esters are exemplified by the reaction product of adipic acid, thioglycol and 2-ethylhexyl mercaptan.

In the preparation of the ester lubricating oils manufacturers are faced with the problem of lowering the final acidity and hydroxyl content of the oil to a point where the synthetic ester lubricant will be acceptable for use in engines at high temperatures. The acidity and hydroxyl content of the synthetic ester lube oil are derived from carboxyl (—COOH) and hydroxyl (—OH) present therein. These radicals are generally always present in crude synthetic ester oils even though in the preparation of the synthetic ester lube the amounts of acid and alcohol reactants are normally proportioned in such a manner that there is equal or near equal number of carboxyl and hydroxyl groups present for reaction with one another. The reasons for the residual amount of free carboxyl and hydroxyl radicals which cause the acidity and hydroxyl content of the synthetic ester lube oil are believed to be three-fold. Firstly, the proportions of alcohol and acid reactants employed may not give an equal number of carboxyl and hydroxyl groups, thereby promoting an excess of one or the other in the ester oil product. Secondly, particularly in commercial preparation of ester lube oils, it is uneconomical from a time standpoint to allow the esterification reaction to go to 100% completion, thus small quantities of unreacted alcohol and acid as well as partially esterified acid and alcohol molecules remain in the final product. Thirdly, although the water by-product is normally continuously removed in ester oil formation, 100% removal is not economically feasible. This residual water causes a small part of the ester oil to hydrolyze to the initial alcohol and acid reactants and/or into partial esters.

The acidity of the synthetic ester lube is detrimental in that it promotes corrosiveness of the lube towards metals. Furthermore, a hydroxyl content in the lube is undesirable in that it enhances the thermal and oxidation instability of the lube.

In the past the residual acidity of ester oils has been reduced by washing with aqueous alkali or by percolating through beds of alkali or alkali impregnated on less active materials. Washing with alkalies, however, frequently results in the formation of stable aqueous emulsions. Although the percolation method may reduce the acidity to the desired point, ester soluble alkali salts of organic acids apparently result since the ester lubricants so treated have been found to possess a high and undesirable ash content. Still further the percolation method has not been found economically desirable since it can result in loss of ester product of approximately 40 to 50%. It has been further proposed to eliminate the acidity of the synthetic ester lubes by using excess alcohol in their preparation. However, this results in a synthetic

lube of a significant hydroxyl content which tends to render it thermally unstable and sensitive to oxidation.

In respect to hydroxyl content it has been proposed to remove the hydroxyl bearing ingredients in a synthetic ester oil by subjecting the ester to fractional distillation under reduced pressure. This procedure was not found effective for reducing hydroxyl content and also caused the ester oil to undesirably darken. The darkening effect is a result of the partial decomposition of the ester oil promoted by the hydroxyl groups therein.

We have discovered and this forms the object of the invention that the acidity and hydroxyl content of crude synthetic ester lubricating oils may be substantially reduced by treatment with an aromatic hydrocarbyl isocyanate or aromatic hydrocarbyl isothiocyanate. We have further found this treatment does not produce the undesirable effects of past methods such as high product loss, emulsion formation and discoloration of the ester oil. The treatment is accomplished by reacting the synthetic ester lube with the isocyanate or isothiocyanates at an elevated temperature, e.g. between about 50 and 250° C. The amounts of aromatic hydrocarbyl isocyanate or isothiocyanate employed to reduce the residual acidity and hydroxyl content of the crude ester will of course depend on the quantity of ester and the quantity of carboxylic and hydroxyl groups therein. However, it has been found that amounts of isocyanate or isothiocyanate between about 0.1 and 10%, preferably between 1 and 5% based on the weight of the ester oil are generally sufficient to reduce neutralization number (Neut. No.) and hydroxyl number (OH No.) of the ester oils prepared by any of the standard methods to desired levels, e.g. to a Neut. No. less than 1 and an OH No. less than 2. It is to be noted Neut. No. and OH No. are respectively relative numerical representations of the carboxyl and hydroxyl concentration in a material.

Under the aforementioned operating conditions the Neut. No. and OH No. of the ester oil can be significantly reduced in a period between about 1 and 20 hrs.

In order to facilitate the reaction of the isocyanate or isothiocyanate with the ester, an inert liquid organic diluent such as toluene and xylene may be employed. Furthermore, under preferred reaction conditions the ester oil and isocyanate or isothiocyanate are continuously mixed under a blanket of inert gas such as nitrogen. The purpose of the inert gas is to insure against possible premature oxidation of the isocyanate or isothiocyanate reactant.

Specific examples of the aromatic hydrocarbyl isocyanates and isothiocyanates contemplated herein are the aryl, alkaryl and aralkyl isocyanates and isothiocyanates of 7 to 30 carbon atoms such as phenyl isocyanate, phenyl isothiocyanate, 4-tolyl isocyanate, 4-tolyl isothiocyanate, 3-phenylbutyl isocyanate, benzyl isocyanate, and benzyl isothiocyanate.

The reaction of the isocyanate or isothiocyanate with the synthetic ester lubricant to reduce its acidity and hydroxyl content has been theorized in the following manner. It is believed that the isocyanate reacts with the carboxyl groups in the synthetic ester to form an amide linkage. In respect to the hydroxyl groups the isocyanate reacts to form a urethane structure. Still further the isocyanate is believed to form a symmetrically disubstituted urea with unremoved water produced in the esterification reaction forming the ester oil. The urethane, amide, and urea products formed in the treatment appear to have some beneficial effect on the properties of the synthetic oil and need not be removed therefrom. However, it is desirable to separate any precipitated products from the ester oil such as by filtration or vacuum stripping.

In a modified procedure of our novel method a stoichiometric excess of alcohol is employed, for example, between about 1 to 10 wt. percent in excess of the amount necessary for the complete esterification of the acid. The crude ester produced under these conditions is of relative-

ly low acidity but has a high hydroxyl content. This high hydroxyl containing ester is treated with isocyanate or isothiocyanate in the manner previously described.

In order to further illustrate the method of the present invention the following examples are given. It is to be understood that these examples are illustrative only and are not considered to be limiting in any way upon the concept of this invention.

#### Example 1

10 In a 5-liter 3-neck flask equipped with a mechanical stirrer, a thermometer and a condenser 134 grams (1.0 mole) of trimethylolpropane, 131 grams (0.65 mole) of sebacic acid, 268 grams (1.7 mole) of pelargonic acid and 50 milliliters of xylene were refluxed for 24 hours at 250° C. During the reaction period 54 mls. of water resulting from the esterification were removed. Analysis of the crude ester product found it to have an OH No. (hydroxyl number) of 10.

20 500 grams of this ester product were admixed with 5 grams of phenyl isocyanate and were heated for 4 hours at 170 to 190° C. The thus treated ester product was analyzed and found to have an OH No. of 0.

#### Example 2

25 To a 12-liter 3-neck flask equipped with a stirrer, two water separators and condensers, 1340 (10 moles) grams trimethylolpropane, 1313 grams (6.5 moles) sebacic acid, 2686 grams (17.0 moles) pelargonic acid, and 300 milliliters of xylene were added. The reaction mixture was refluxed for 22 hours at a temperature of 255-275° C. At the end of the reaction period 535 milliliters of water or over 99% of the theoretical amount of water resulting from complete esterification was removed. The Neut. No. of the crude ester product was 3.5.

30 The ester product was cooled to 200° C. and while bubbling nitrogen through the product to form a blanket of nitrogen thereover, 53 grams of phenyl isocyanate was added over a period of 5 minutes. The ester product and isocyanate were held at said temperature with mixing for a period of 6 hours. At the end of the 6 hour period the thus treated ester was analyzed, found to have a Neut. No. of 0.32. The treated ester (wt. 4923 grams) was filtered to remove small amounts of crystalline diphenylurea and was stripped to 230° C. at 15 mm. Hg pressure for one hour. The stripped ester weighed 4505 grams (94.5% molar yield) and had a Neut. No. of 0.10, a kinematic viscosity at 210° F. of 47.2 cs. and a pour point of minus 25° F.

#### Example 3

35 The esterification and phenyl isocyanate treatment procedures of Example 2 were repeated except 1366 grams (10.2 moles) of trimethylolpropane, 1313 grams (6.5 moles) sebacic acid and 2686 grams (17.0 moles) pelargonic acid were employed thereby forming an esterification reaction mixture containing a 2 mole percent alcohol excess on an equivalent basis over the total acid reactants. In addition 54 grams of phenyl isocyanate were employed. At the end of the ester-forming reaction period the crude synthetic lubricant had a Neut. No. of 1.8. After the phenyl isocyanate treatment the stripped product had a Neut. No. of 0.1.

#### Example 4

40 To a 12-liter, 3-neck flask equipped with a stirrer, a thermometer and a dropping funnel there were charged 8770 grams of a complex ester of a Neut. No. of 3.7 resulting from the reaction of trimethylolpropane, pelargonic acid and sebacic acid. Nitrogen was bubbled through the material which was heated with stirring. When the pot temperature reached 200° C., 100 grams of phenyl isocyanate were added dropwise through the dropping funnel. Heating was continued for 12 hrs. at 190-200° C. At the end of the 12 hour period the ester was analyzed and found to have a Neut. No. of 0.8. Subsequently

the isocyanate treated ester was stripped at 230° C.-10 mm. Hg and crystalline diphenylurea formed during the isocyanate treatment was removed by filtration. The Neut. No. of this finished ester product was 0.3.

We claim:

1. A method for reducing the acidity and hydroxyl content of a synthetic ester lubricating oil derived from the esterification of a hydrocarbyl carboxylic acid with a hydrocarbyl alcohol and containing unesterified substituent groups derived from said esterification, said substituent groups selected from the group consisting of unesterified free carboxylic acid groups, unesterified free alcohol groups and mixtures thereof comprising contacting said synthetic ester lubricating oil containing said unesterified free substituent groups with an aromatic compound of 7 to 30 carbons selected from the group consisting of phenyl monoisoxyanate, phenylalkyl monoisoxyanate, alkylphenyl monoisoxyanate, phenyl monoisoxyanate, phenylalkyl monoisoxyanate, and alkylphenyl monoisoxyanate at a temperature between about 50 and 250° C. so as to react said aromatic compound with said unesterified free substituent groups, said aromatic compound being present in a proportion between about 0.1 and 10 wt. percent of said ester lubricating oil.

2. A method for reducing the acidity and hydroxyl content of a synthetic ester lubricating oil derived from the esterification of hydrocarbyl alcohol with hydrocarbyl carboxylic acid and containing unesterified free substituent groups derived from said esterification, said substituent groups selected from the group consisting of unesterified free carboxylic acid groups and unesterified free alcohol groups and mixtures thereof comprising contacting said ester lubricating oil containing said unesterified free substituent groups in an atmosphere of inert gas with from 1 to 5 wt. percent phenyl monoisoxyanate based on the weight of said lubricating oil at a temperature between about 50 and 250° C. so as to react said aromatic compound with said unesterified free substituent groups.

3. A method for reducing the acidity and hydroxyl content of a synthetic ester lubricating oil derived from

the esterification of hydrocarbyl carboxylic acid with hydrocarbyl alcohol and containing unesterified free substituent groups derived from said esterification, said substituent groups selected from the group consisting of unesterified free carboxylic acid groups and unesterified free alcohol groups and mixtures thereof wherein said oil was formed with between 1 and 10 wt. percent stoichiometric excess of said hydrocarbyl alcohol comprising contacting said ester lubricating oil containing said unesterified free substituent groups with an aromatic compound of 7 to 30 carbons selected from the group consisting of phenyl monoisoxyanate, phenylalkyl monoisoxyanate, alkylphenyl monoisoxyanate, phenyl monoisoxyanate, phenylalkyl monoisoxyanate, and alkylphenyl monoisoxyanate at a temperature between about 50 and 250° C. so as to react said aromatic compound with said unesterified free substituent groups, said aromatic compound being present in a proportion of 0.1 and 10 wt. percent based on said oil.

5 20. 4. A method in accordance with claim 2 wherein said ester lubricating oil is a complex ester lubricating oil resulting from the reaction of trimethylolpropane, sebacic acid and pelargonic acid, and said inert gas is nitrogen.

5 25. 5. A method in accordance with claim 2 wherein said ester lubricating oil is a complex ester lubricating oil resulting from reaction of trimethylolpropane, sebacic acid and 2-ethylhexanol and said inert gas is nitrogen.

5 30. 6. A method in accordance with claim 3 wherein said ester lubricating oil is a complex ester lubricating oil resulting from the reaction of trimethylolpropane, sebacic acid and pelargonic acid.

#### References Cited by the Examiner

##### UNITED STATES PATENTS

35 2,861,981 11/58 Frank et al. ----- 260-485  
3,053,871 9/62 Aries ----- 260-448

##### FOREIGN PATENTS

40 738,254 7/43 Germany.

CHARLES B. PARKER, Primary Examiner.

T. E. LEVOW, L. ZITVER, Examiners.